# EUROPEAN PATENT SPECIFICATION

(11) **EP 3 269 934 B1**
(45) Date of publication and mention of the grant of the patent: **30.08.2023**
(21) Application number: 17180782.9
(22) Date of filing: 11.07.2017
(51) Int. Cl.: F01D 5/28, F01D 25/00, C23C 4/04, C23C 28/00

(54) **STRUCTURE COMPRISING A REFLECTIVE THERMAL BARRIER COATING AND CORRESPONDING METHOD OF CREATING A THERMAL BARRIER COATING**
STRUKTUR MIT EINER REFLEKTIERENDEN WÄRMEDÄMMSCHICHT UND ZUGEHÖRIGES VERFAHREN ZUR HERSTELLUNG EINER WÄRMEDÄMMSCHICHT
STRUCTURE AYANT UN REVÊTEMENT RÉFLECHISSANT DE BARRIÈRE THERMIQUE ET PROCÉDÉ DE FABRICATION D'UN REVÊTEMENT DE BARRIÈRE THERMIQUE

(30) Priority: 12.07.2016 US 201615208066
(43) Date of publication of application: 17.01.2018
(73) Proprietor: Collins Engine Nozzles, Inc., West Des Moines, IA 50265 (US)
(72) Inventor: STAROSELSKY, Alexander, Avon, CT 06001 (US); MARTIN, Thomas J., East Hampton, CT 06424 (US)
(74) Representative: Dehns

(56) References cited:
- EP-A1- 3 088 559
- DE-A1-102009 015 154
- US-A- 4 916 022
- US-A1- 2011 280 717
- US-B1- 6 210 791
- US-B1- 6 465 090

## Description

### BACKGROUND

### 1. Field

The present invention relates to thermal barrier coatings, more specifically to a structure for use in a high temperature environment, the structure comprising a thermal barrier coating, and to a method for creating a thermal barrier coating.

### 2. Description of Related Art

In modern turbomachines, which comprise turbofans, turbojets, gas turbine engines, and the like, the purpose of the turbine component is to extract work from the high pressure and high temperature core flow. The two most important parameters that determine the turbine's power output and fuel efficiency are the rotor speed and combustion temperature. Increases in the rotor speed and combustion temperature offer the greatest improvements to the fuel efficiency and power output of the engine. It is well understood that the turbine rotor speed determines the maximum pressure ratios that can be obtained by the turbine, and increasing the speed, temperature and cross-sectional area of the core flow increases the amount of energy that can be extracted as work to drive the fan and compressor. As a consequence, hot section components, such as combustor liners, turbine airfoils, and air seals, are subjected to the highest possible temperatures, which result in increased risk of structural failure, and accelerated material deterioration and degradation due to creep, oxidation, corrosion and thermo-mechanical fatigue at high temperature.

Thermal barrier coatings (TBC), shield the hot section components from the high temperature external gases, providing up to 400 degrees C protection, which allows the turbine components to be fully operable and durable at higher temperatures, providing greater power and fuel efficiency. The structural performance and life capabilities of hot section components rely on this TBC property. The current TBC material for gas turbine hot section components is yttria partially stabilized zirconia (YPSZ or YSZ). Zirconia (ZrO2) has good erosion resistance, a lower intrinsic thermal conductivity and most suitable thermal expansion coefficient as compared to other ceramics such as alumina (Al2O3). Yttria (Y2O3) is added into pure zirconia to stabilize the cubic or tetragonal structure and further reduce the thermal conductivity. In addition to the chemical composition, the method of processing and structure of the coating has a significant impact on the thermal and mechanical properties of the coating. However, the capability of these zirconia based materials is still limited. Zirconia-based TBCs are only partially transparent to infrared (thermal) radiation.

Increase of the combustion gas temperature causes significant increase of the amount of heat transferred from the gas via infrared radiation, because it is proportional to the temperature in the fourth power. The absorbance of zirconia-based thermal barrier coatings to infrared radiation reduces dramatically with wavelengths shorter than 8 µm, and becoming almost fully transparent below 4 µm. The reflectance of TBCs in the IR range of 1 to 4 µm is also low (about 0.2) for single crystal (EB-PVD) TBCs, but better for thermal spray TBCs (0.5) due to increased scattering, which increases with increasing temperature. Therefore, zirconia-based TBCs provide only poor protection to surfaces exposed to the intense thermal radiation of the combustion in the engine. This is made worse by the fact that the peak blackbody radiation intensity is around 2.5 µm at convectional engine operating temperatures, making YSZ TBC protection versus thermal radiation lesser with increasing engine operating temperatures.

Such conventional thermal protection systems have generally been considered satisfactory for their intended purpose. However, there is still a need in the art for improved thermal barrier coatings. The present invention provides a solution for this need.

DE102009015154 discloses a ceramic material which contains infrared-reflecting metal components. US2011280717 discloses a structure with the features of the preamble of claim 1. US6465090 discloses a protective coating and coating method for protecting a thermal barrier coating. US6210791 discloses a coated article comprising a diffuse reflective barrier. US 4916022 discloses a ceramic thermal barrier coating system for superalloy components subjected to high operating temperatures.

### SUMMARY

A structure (e.g. a structure produced by the method as herein described) for use in a high temperature environment includes (e.g. comprises) a substrate and a thermal barrier coating disposed on the substrate comprising a base material and one or more reflective layers disposed in the base material, each reflective layer having a plurality of reflective particulates. The volume fraction of the reflective particulates is 2% to 5% of the total volume of the thermal barrier coating. The reflective particulates include a material that reflects wavelengths below about 8 microns. The reflective particulates include TiO₂ particulates.

The structure can be a turbine blade, and/or the base material of the thermal barrier coating can be yttria-stabilized zirconia, for example.

The substrate can include a metal alloy (e.g. a nickel alloy). Any other suitable material is contemplated herein for the substrate. The base material can include a ceramic material (e.g., that inherently has a low absorbance and reflectance of infrared radiation). Any other suitable material is contemplated herein.

The reflective particulates can include at least one of a spherical shape, a conical shape, an elliptical shape, a spheroid shape, or a fiber.

Reflective particles can be substantially smaller than the thickness of the thermal barrier coating. The volume fraction of the reflective particulates may include reflective particulates that are less than about 4 microns in diameter and in length.

The one or more reflective layers can include a plurality of reflective layers, each reflective layer separated by about 1 to about 3 lengths of the reflective particulates. Any other suitable separation is contemplated herein.

In certain embodiments, the one or more reflective layers can be located no deeper than about 25% of a thickness of the thermal barrier coating from a surface of the thermal barrier coating.

The invention also provides a method (e.g. a method for producing a structure as herein described) for creating a thermal barrier coating comprising applying a base material to a substrate and disposing one or more reflective layers having a plurality of reflective particulates within the base material. The volume fraction of the reflective particulates is 2% to 5% of the total volume of the thermal barrier coating. The reflective particulates include a material that reflects wavelengths below about 8 microns. The reflective particulates include TiO₂ particulates.

Applying the base material can include thermal spraying or cold spraying the substrate with the base material.

Disposing one or more reflective layers can include thermal spraying or cold spraying the base material with reflective particulates. Applying and disposing can be at least partially simultaneously performed by spraying the substrate or the base material with a slurry including the base material and the reflective particulates.

These and other features of the systems and methods of the subject invention will become more readily apparent to those skilled in the art from the following detailed description taken in conjunction with the drawings.

### BRIEF DESCRIPTION OF THE DRAWINGS

So that those skilled in the art to which the subject invention appertains will readily understand how to make and use the devices and methods of the subject invention without undue experimentation, embodiments thereof will be described in detail herein below with reference to certain figures, wherein:
Fig. 1 is a partial cross-sectional view of an embodiment of a structure in accordance with this invention; and
Fig. 2 is a partial perspective view of an embodiment of a thermal barrier coating in accordance with this invention.

### DETAILED DESCRIPTION

Reference will now be made to the drawings wherein like reference numerals identify similar structural features or aspects of the subject invention. For purposes of explanation and illustration, and not limitation, an illustrative view of an embodiment of a structure in accordance with the invention is shown in Fig. 1 and is designated generally by reference character 100.

Other embodiments and/or aspects of this invention are shown in Fig. 2. The systems and methods described herein can be used to improve the usable life of structures (e.g., turbine blades) exposed to high heat environments (e.g., in turbomachines), for example.

Referring to Fig. 1, a structure 100 includes a substrate 101 and a thermal barrier coating 103. The thermal barrier coating 103 includes a base material 105 and one or more reflective layers 107 disposed in the base material 103. Each reflective layer has a plurality of reflective particulates 109 (e.g., infrared reflective particles).

The structure 100 can be a turbine blade (e.g., for a turbomachine), for example. Any other suitable structure for use in a high temperature environment is contemplated herein.

The substrate 101 can include a nickel alloy. Any other suitable material is contemplated herein for the substrate 101. The base material 105 can include a ceramic material (e.g., yttria partially stabilized zirconia). Any other suitable material is contemplated herein.

The reflective particulates 109 include a material that reflects wavelengths in the short and mid wavelength infrared spectrum. The reflective particulates reflect wavelengths below about 8 microns (e.g., less than 4 microns).

The reflective particulates can be configured to reflect thermal radiation to a greater extent than the base material in at least a certain range of wavelengths. The reflective particulates include TiO₂ particulates which have increased reflectance in the short and mid infrared wavelengths over yttria partially stabilized zirconia.

The reflective particulates 109 can include at least one of a spherical shape, a conical shape, an elliptical shape, a spheroid shape, or a fiber, rhombohedral, for example. The reflectivity can change and/or be selected based on the particle shape. For example, there exists in general such a relation of scattering cross sections: C sphere <Cneedle < Cdisc. Moreover, the reflective particulates can be sized to include suitable electromagnetic properties to reflect energy of a desired wavelength or range of wavelengths (e.g., having a diameter less than one-half the wavelength of light to be scattered, such as a diameter of about 0.5 microns to about 4 microns). Any suitable shape and/or size of the reflective particulates 109 and/or combinations thereof in a single or multiple layers 107 is contemplated herein.

The volume fraction of the reflective particulates 109 is 2% to 5% of total volume of the thermal barrier coating 103 depending on their scattering efficiency. For example, a volume fraction of spherical reflective particulates 109 of about 2.75% with rhombohedral arrangement of the reflective particulates can provide about 50% scattering efficiency. The reflective particulates 109 having a fiber shape may demonstrate better performance.

Referring additionally to Fig. 2, the one or more reflective layers 107 can include a plurality of reflective layers 107 (e.g., a first layer 107a disposed under a second layer 107b in thermal barrier coating 203). Each layer 107a, 107b can include any suitable reflective particulates 109 (e.g., of different shape, of the same shape, or of any suitable combination of shapes). Each reflective layer 107 can be separated by about 1 to about 3 lengths of the reflective particulates 109. Any other suitable separation is contemplated herein.

In certain embodiments, the one or more reflective layers 107 can be located no deeper than about 25% (e.g., less than 5%) of a thickness of the thermal barrier coating 103 from a surface of the thermal barrier coating 105. In this regard, the reflective particulates 109 can be localized near the surface of the thermal barrier coating 103. Any other suitable depth for reflective particulates 109 is contemplated herein.

A distribution density of reflective particulates 109 in the base material 105 can be selected to maximize reflectivity without compromising thermal conductivity or structural stability of the thermal barrier coating 103, for example. Embedded reflective particulates (e.g., fibers) can be disposed to generate an irregular grid submerged in the infrared transparent matrix of the base material 105 that generates the composite structure which effectively reflects the incident light 111. Any other suitable distribution density and/or pattern thereof is contemplated herein.

In accordance with at least one aspect of this invention, a method for creating a thermal barrier coating with the features of independent claim 9 is disclosed. Applying the base material 105 can include thermal spraying or cold spraying the substrate 101 with the base material 105.

Disposing one or more reflective layers 107 can include thermal spraying or cold spraying the base material 105 with reflective particulates 109. Applying and disposing can be at least partially simultaneously performed by spraying the substrate 101 or the base material 105 with a slurry that has both the base material 105 and the reflective particulates 109, for example. While described as layers 107 above, demarcation is not necessary because the thermal barrier coating can be continuous such that particulates 109 are disposed within continuously formed base material 105 during formation of the thermal barrier coating.

As described above, in order to reflect a targeted range of wavelengths, layers of ceramic materials with low and high refractive indices can be added without deteriorating the thermal barrier coating structural properties. A broadband reflection of the infrared (e.g., low and/or medium wave) wavelengths can be achieved by the selection of the corresponding size of the reflecting elements. Infrared reflection can reduce the temperature up to 160 degrees F (90 degrees C) on the metal interface surface between the substrate 101 and the thermal barrier coating 103 that eventually leads to up to a fivefold lifetime increase for turbine blades, for example.

In the layers 107 having high refractive index particles, infrared light is bent with the result that light travels a shorter path in the coating and does not penetrate through it causing practically all incident light 111 to be returned to the surface as reflected light 113. Effective scattering can be achieved if the particles diameter is slightly less than one-half the wavelength of light to be scattered, for example.

Certain embodiments utilize the reflective properties of TiO₂ fibers and/or particles together with their thermal and oxidation stability. TiO₂ fibers, for example, can impart structural enhancements to the ceramic thermal barrier coating exhibiting a structure similar to ferro-concrete. The fibers can enhance the material's toughness while maintaining or even enhancing its thermal and environmental insulating properties. For example, the reinforced composite material has been found to have up to 5 times the fracture toughness over monolithic ceramic materials fabricated with the same process, especially when the material is subject to cyclic loadings.

Embodiments provide the ability of a thermal barrier coating that effectively reflects thermal radiation over a wide spectral range which can significantly improve the efficiency of thermal barrier coatings. For turbomachine parts, improved reflectance leads to extension of part life and to the increase of overall turbine efficiency, for example. Current methods to increase hot section parts durability only address the convective portion of the heat load. Further, at higher temperature, a great portion of the heat transferred to the part has radiative nature and not convective heat. Existing thermal barrier coatings only address the convective portion of the heat load because they are almost transparent to the radiative portion at the wavelength of peak flux.

The methods and systems of the present invention, as described above and shown in the drawings, provide for thermal barrier coatings with superior properties including improved reflectance.

## Claims

1. A structure (100) for use in a high temperature environment, comprising:
a substrate (101); and
a thermal barrier coating (103, 203) disposed on the substrate comprising a base material (105) and one or more reflective layers (107) disposed in the base material (105); each reflective layer (107) having a plurality of reflective particulates (109);
the reflective particulates (109) including a material that reflects wavelengths below 8 microns;
the reflective particulates (109) including TiO₂ particulates;
**characterized in that**:
the volume fraction of the reflective particulates (109) is 2% to 5% of total volume of the thermal barrier coating (103, 203).

2. The structure (100) of claim 1, wherein the substrate (101) includes a metal alloy.

3. The structure (100) of claim 1 or claim 2, wherein the base material (105) includes a ceramic material.

4. The structure (100) of any preceding claim, wherein the reflective particulates (109) include at least one of a spherical shape, a conical shape, an elliptical shape, a spheroid shape, or a fiber.

5. The structure (100) of any preceding claim, wherein the base material (105) of the thermal barrier coating (103, 203) is yttria-stabilized zirconia.

6. The structure (100) of any preceding claim, wherein the one or more reflective layers (107) includes a plurality of reflective layers (107), each reflective layer (107) separated by 1 to 3 lengths of the reflective particulates (109).

7. The structure (100) of any preceding claim, wherein the one or more reflective layers (107) are located no deeper than 25% of a thickness of the thermal barrier coating (103, 203) from a surface of the thermal barrier coating (103, 203).

8. The structure (100) of any preceding claim, wherein the structure (100) is a turbine blade.

9. A method for creating a thermal barrier coating (103, 203), comprising:
applying a base material (105) to a substrate (101); and
disposing one or more reflective layers (107) having a plurality of reflective particulates (109) within the base material (105),
wherein the volume fraction of the reflective particulates (109) is 2% to 5% of total volume of the thermal barrier coating (103, 203);
the reflective particulates (109) include a material that reflects wavelengths below 8 microns; and
the reflective particulates (109) include TiO₂ particulates.

10. The method of claim 9, wherein applying the base material (105) includes thermal spraying or cold spraying the substrate with the base material (105).

11. The method of claim 9 or claim 10, wherein disposing one or more reflective layers (107) includes thermal spraying or cold spraying the base material (105) with reflective particulates (109).

12. The method of any one of claims 9-11, wherein applying and disposing are at least partially simultaneously performed by spraying the substrate (101) or the base material (105) with a slurry including the base material (105) and the reflective particulates (109).

## Patentansprüche

1. Struktur (100) zur Verwendung in einer Hochtemperaturumgebung, umfassend:
ein Substrat (101); und
eine Wärmedämmschicht (103, 203), die auf dem Substrat angeordnet ist und ein Basismaterial (105) und eine oder mehrere reflektierende Schichten (107), die in dem Basismaterial (105) angeordnet sind, umfasst;
wobei jede reflektierende Schicht (107) eine Vielzahl von reflektierenden Teilchen (109) aufweist;
wobei die reflektierenden Teilchen (109) ein Material beinhalten, das Wellenlängen unter 8 Mikrometer reflektiert;
wobei die reflektierenden Teilchen (109) TiO₂-Teilchen beinhalten;
**dadurch gekennzeichnet, dass**:
der Volumenanteil der reflektierenden Teilchen (109) 2 % bis 5 % des Gesamtvolumens der Wärmedämmschicht (103, 203) beträgt.

2. Struktur (100) nach Anspruch 1, wobei das Substrat (101) eine Metalllegierung beinhaltet.

3. Struktur (100) nach Anspruch 1 oder Anspruch 2, wobei das Basismaterial (105) ein Keramikmaterial beinhaltet.

4. Struktur (100) nach einem der vorhergehenden Ansprüche, wobei die reflektierenden Teilchen (109) mindestens eines von einer Kugelform, einer konischen Form, einer elliptischen Form, einer Sphäroidform oder einer Faser beinhalten.

5. Struktur (100) nach einem der vorhergehenden Ansprüche, wobei das Basismaterial (105) der Wärmedämmschicht (103, 203) mit Yttriumoxid stabilisiertes Zirkoniumoxid ist.

6. Struktur (100) nach einem der vorhergehenden Ansprüche, wobei die eine oder die mehreren reflektierenden Schichten (107) eine Vielzahl von reflektierenden Schichten (107) beinhalten, wobei jede reflektierende Schicht (107) durch 1 bis 3 Längen der reflektierenden Teilchen (109) getrennt ist.

7. Struktur (100) nach einem der vorhergehenden Ansprüche, wobei sich die eine oder die mehreren reflektierenden Schichten (107) nicht tiefer als 25 % einer Dicke der Wärmedämmschicht (103, 203) von einer Oberfläche der Wärmedämmschicht (103, 203) befinden.

8. Struktur (100) nach einem der vorhergehenden Ansprüche, wobei die Struktur (100) eine Turbinenschaufel ist.

9. Verfahren zum Herstellen einer Wärmedämmschicht (103, 203), umfassend:
Aufbringen eines Basismaterials (105) auf ein Substrat (101); und
Anordnen einer oder mehrerer reflektierender Schichten (107) mit einer Vielzahl von reflektierenden Teilchen (109) innerhalb des Basismaterials (105),
wobei der Volumenanteil der reflektierenden Teilchen (109) 2 % bis 5 % des Gesamtvolumens der Wärmedämmschicht (103, 203) beträgt;
wobei die reflektierenden Teilchen (109) ein Material beinhalten, das Wellenlängen unter 8 Mikrometer reflektiert; und
wobei die reflektierenden Teilchen (109) TiO₂-Teilchen beinhalten.

10. Verfahren nach Anspruch 9, wobei das Aufbringen des Basismaterials (105) thermisches Spritzen oder Kaltgasspritzen des Substrats mit dem Basismaterial (105) beinhaltet.

11. Verfahren nach Anspruch 9 oder Anspruch 10, wobei das Anordnen einer oder mehrerer reflektierender Schichten (107) thermisches Spritzen oder Kaltgasspritzen des Basismaterials (105) mit reflektierenden Teilchen (109) beinhaltet.

12. Verfahren nach einem der Ansprüche 9-11, wobei das Aufbringen und Anordnen zumindest teilweise gleichzeitig durch Spritzen des Substrats (101) oder des Basismaterials (105) mit einer Aufschlämmung durchgeführt werden, die das Basismaterial (105) und die reflektierenden Teilchen (109) beinhaltet.

## Revendications

1. Structure (100) destinée à être utilisée dans un environnement à haute température, comprenant :
un substrat (101) ; et
un revêtement de barrière thermique (103, 203) disposé sur le substrat comprenant un matériau de base (105) et une ou plusieurs couches réfléchissantes (107) disposées dans le matériau de base (105) ;
chaque couche réfléchissante (107) ayant une pluralité de particules réfléchissantes (109) ;
les particules réfléchissantes (109) comportant un matériau qui réfléchit les longueurs d'onde inférieures à 8 microns ;
les particules réfléchissantes (109) comportant des particules de TiO₂ ;
**caractérisée en ce que** :
la fraction volumique des particules réfléchissantes (109) est de 2 % à 5 % du volume total du revêtement de barrière thermique (103, 203).

2. Structure (100) selon la revendication 1, dans laquelle le substrat (101) comporte un alliage métallique.

3. Structure (100) selon la revendication 1 ou la revendication 2, dans laquelle le matériau de base (105) comporte un matériau céramique.

4. Structure (100) selon une quelconque revendication précédente, dans laquelle les particules réfléchissantes (109) comportent au moins l'une d'une forme sphérique, d'une forme conique, d'une forme elliptique, d'une forme sphéroïdale ou d'une fibre.

5. Structure (100) selon une quelconque revendication précédente, dans laquelle le matériau de base (105) du revêtement de barrière thermique (103, 203) est de la zircone stabilisée à l'yttrium.

6. Structure (100) selon une quelconque revendication précédente, dans laquelle les une ou plusieurs couches réfléchissantes (107) comportent une pluralité de couches réfléchissantes (107), chaque couche réfléchissante (107) étant séparée par 1 à 3 longueurs de particules réfléchissantes (109).

7. Structure (100) selon une quelconque revendication précédente, dans laquelle les une ou plusieurs couches réfléchissantes (107) ne sont pas situées à plus de 25 % d'une épaisseur du revêtement de barrière thermique (103, 203) à partir d'une surface du revêtement de barrière thermique (103, 203) .

8. Structure (100) selon une quelconque revendication précédente, dans laquelle la structure (100) est une aube de turbine.

9. Procédé de création d'un revêtement de barrière thermique (103, 203), comprenant :
l'application d'un matériau de base (105) sur un substrat (101) ; et
la disposition d'une ou de plusieurs couches réfléchissantes (107) ayant une pluralité de particules réfléchissantes (109) à l'intérieur du matériau de base (105),
dans lequel la fraction volumique des particules réfléchissantes (109) est de 2 % à 5 % du volume total du revêtement de barrière thermique (103, 203) ;
les particules réfléchissantes (109) comportent un matériau qui réfléchit les longueurs d'onde inférieures à 8 microns ; et
les particules réfléchissantes (109) comportent des particules de TiO₂.

10. Procédé selon la revendication 9, dans lequel l'application du matériau de base (105) comporte une pulvérisation thermique ou une pulvérisation à froid du substrat avec le matériau de base (105).

11. Procédé selon la revendication 9 ou la revendication 10, dans lequel la disposition d'une ou de plusieurs couches réfléchissantes (107) comportent une pulvérisation thermique ou une pulvérisation à froid du matériau de base (105) avec des particules réfléchissantes (109).

12. Procédé selon l'une quelconque des revendications 9 à 11, dans lequel l'application et la disposition sont réalisées au moins partiellement simultanément en pulvérisant le substrat (101) ou le matériau de base (105) avec une barbotine comportant le matériau de base (105) et les particules réfléchissantes (109) .
